

Nov. 7, 1939.

G. N. PIFER

2,178,896

PROCESS OF MAKING PHOTOGRAPHS

Original Filed Aug. 7, 1935



INVENTOR.

GEORGE N. PIFER

BY

Kris Hudson & Kent  
ATTORNEYS

## UNITED STATES PATENT OFFICE

2,178,896

## PROCESS OF MAKING PHOTOGRAPHS

George N. Pifer, Cleveland Heights, Ohio, assignor to Speedtype, Inc., Cleveland, Ohio, a corporation of Ohio.

Application August 7, 1935, Serial No. 35,068  
Renewed April 11, 1939

2 Claims. (Cl. 95—88)

This invention relates to a process of making photographs by the atomizing or spraying method, and has particular reference to a process for use in automatic photographing machines having the atomizing and spraying features disclosed in my prior Patents Nos. 1,682,931, 1,728,361, and 1,751,881, and in my pending application filed December 5, 1934, Serial No. 756,098, the present invention being an improvement over the method 10 and the manipulation of chemicals in developing the photographic image.

Positive images are produced in automatic photographing machines by two well known methods, viz., the exposed sensitized surface is developed into a negative image which is reversed into a positive by removing the developed portions with acids which will not affect the unaltered or unexposed portions, the latter then being again exposed to actinic light and redeveloped, or the latter may be transformed by the well known sulphide method without the aid of reexposure to light by treating the unreduced silver portions with a sulphide solution, which produces the final and positive image.

The objects of the present invention or of my improved method are, first, to eliminate the reexposure to light, and, second, to eliminate the use of the sulphide solution with its contaminating characteristics and to substitute a chemical 30 fogging or blackening action to produce the final image.

In my pending application above referred to, there is disclosed in the atomizing and spraying device or mechanism a mixing cell and mechanical means by which the different solutions in atomized condition can be superposed upon each other in quick succession. This mechanism and the method utilized therewith are preferably employed in carrying out the present invention.

As is well known, the usual manipulation in reversing a negative image into a positive picture includes the use of an alkaline developer, an acid with an oxidizing agent, and a sulphite of soda clearing solution which is applied after the bleaching action of the acid to remove the discolored produced by the acid. In common practice, where the exposed sensitized card surface is immersed in successive baths, it is essential to wash or rinse the surface between the several immersions so as not to contaminate one solution with the other or else the staining or fogging action will result and the solutions will deteriorate. It is precisely this fogging action which is here used to redevelop the positive image, on the one hand dispensing with the re-

exposure to light, and on the other hand, the contaminating sulphur and sulfid treatment. This, in turn, necessarily reduces the washing and the rinsing operations, and, with the aid of the aerated developing solutions discharged from the nozzle of the atomizer, speeds up the manipulation for quick completion of the positive picture and its delivery from the automatic photographing machine if the invention is used in connection therewith.

My improved process is as follows:

When the exposed sensitized surface (which may be any of the usual silver salts, such as bromide of silver) is first developed, the atomizer next applies a quick superficial wash. Then there is applied a diluted solution of sulphuric acid and a suitable oxidizing agent, such as permanganate of potash or bichromate of potash, to remove the developed image, followed by a quick superficial rinse, if desired, and then a suitable stain removing solution is quickly applied, such as a "hypo" solution of sodium thiosulphate; while there still remains traces of "hypo" on the surface of the film which already is permeated with acid and the oxidizing agent, the developer is again quickly applied, and this, by combining with the traces of the acid solution and "hypo", chemically fogs, blackens, and redevelops the remaining bromide of silver without reexposure to light. Preferably there is no intervening wash between the application of the clearing solution and the second application of the developer.

The process will be more clearly understood in connection with the accompanying drawing which shows diagrammatically how the atomizing or spraying equipment may be used advantageously in applying the different solutions to the exposed sensitized surface.

The solutions are supplied from suitable receptacles designated 1, 2, 3, and 4 which are connected by flexible tubes A, B, C, and D to a mixing chamber or cell 5 having an outlet 5a. Air is supplied from a conduit 6 connected to a pressure pump through a nozzle 7 which is arranged in proximity to the orifice at the upper end of the outlet 5a of the cell so as to direct a stream of air immediately over and across the orifice of the outlet. The receptacles 1, 2, 3, and 4 may be assumed to contain, respectively, the developer, water, the acid bleach, and the "hypo."

Normally, the flexible tubes A, B, C, and D are closed by any suitable mechanical closing means, and whenever a solution is to be drawn from a receptacle into the cell and discharged in a spray or aerated condition onto the exposed sensitized

surface, which is designated 8, the closing means for the tube leading to a given receptacle is released from the tube so as to allow the solution to be drawn up through the tube into the cell by the suction created by the stream of air passing from the nozzle 7. Then the tube is again immediately closed. If the present process is used in an automatic photographing machine, I prefer to use for opening and closing the tubes the mechanism shown in my application Serial No. 756,098, this mechanism including cam controlled rollers which move in one direction to compress and close the tubes and in the reverse direction to open them. In the accompanying drawing the opening and closing means is indicated conventionally by an ordinary hand manipulated clip designated 9 one of which can be applied to each tube.

It is obvious that, if the closing means for only one of the solution tubes is released, that one solution only is applied to the sensitized surface, but if more than one closing means is released or set free at the same time, the solutions from the corresponding receptacles will be drawn up into the mixing chamber and there intermixed, and in that mixed condition will be applied to the sensitized surface.

To make a picture by my improved reversing method, assuming that the film or card containing the sensitized medium has been exposed and automatically or otherwise placed in developing position with reference to the nozzle 7, tube A connected to receptacle 1 containing the developing solution, which is the usual alkaline developer, is released for application onto the sensitized surface of the film or card in the form of an atomized spray. One of the developers which might be used in carrying out my improved reversing method consists of the following:

|    |                                                                            |        |     |
|----|----------------------------------------------------------------------------|--------|-----|
| 40 | Caustic soda                                                               | ounces | 1½  |
|    | Sulphite of soda                                                           | do     | 4   |
|    | Hydroquinone                                                               | do     | 1   |
|    | Metol (mono-methyl-para-amino-phenol-sulphate) $(CH_3NHC_6H_4OH)_2H_2SO_4$ | grams  | 160 |
| 45 | Potassium bromide                                                          | do     | 80  |
|    | Water                                                                      | ounces | 64  |

When the surface is sufficiently far developed, tube A is closed, and tube B is opened, causing water to be drawn from receptacle 2 and applied to the surface as a spray, thus giving the surface a quick rinse. The solution from receptacle 3 containing the acid and oxidizing agent to remove the developed image is then released and sprayed onto the surface, and this solution at the same time permeates the entire film and leaves it in an acidified condition before the tube C is shut off. Then tube D is opened to release the

"hypo" solution from receptacle 4 which is then sprayed or atomized onto the sensitized surface and, simultaneously or before the "hypo" is actually shut off, the tube leading from receptacle 1 is again opened or released, causing developing solution to be again sprayed onto the surface 8 to redevelop the image. Then the rinsing spray is again applied to the surface after the tube supplying the second application of developer has been shut off or closed and the positive picture is completed.

It will be seen that by this modus operandi or manipulation the second development takes place in the presence of the "hypo" which is still present in the mixing cell. That is to say, a mixture of the developer and the "hypo" is applied to the film or sensitized surface, and this application of the developer with some of the "hypo" is made onto the sensitized surface with the latter still in an acidified condition. This produces a blackening or fogging action on the unreduced salt remaining in the sensitized surface without a second exposure to light, and this forms or constitutes the final and positive image.

While I have explained the preferred method of carrying out the invention and certain preferred chemicals, I do not desire to be confined to the precise details of the process nor to the particular chemicals mentioned, but aim in my claims to cover all modifications which do not involve a departure from the spirit and scope of the invention in its broadest aspects.

Having thus described my invention, I claim:

1. The process of producing a photograph which comprises applying a developing solution to the exposed sensitized surface, then applying an acid bleaching solution thereto, partially removing said bleaching solution, then applying a "hypo" solution, and then without an intervening washing of the surface and while the same is in an acid condition and without exposure to light, applying a developing solution thereto in the presence of the "hypo" solution which mixes with the developing solution and acts as an accelerator therefor.

2. The process of producing a photograph which comprises applying a developing solution to the exposed sensitized surface, then applying an acid bleaching solution thereto, partially removing said bleaching solution, then applying a "hypo" solution to said surface by atomization, and then without an intervening washing of the surface and while the same is in an acid condition and without exposure to light applying a developing solution thereto in the presence of the "hypo" solution which mixes with the developing solution and acts as an accelerator therefor.

GEORGE N. PIFER.